

# UNITED STATES PATENT OFFICE.

CARL T. FULLER, OF NUTLEY, NEW JERSEY, ASSIGNOR TO GENERAL ELECTRIC COMPANY, A CORPORATION OF NEW YORK.

## TREATMENT OF TUNGSTEN FILAMENTS.

1,280,704.

Specification of Letters Patent.

Patented Oct. 8, 1918.

No Drawing.

Application filed April 13, 1914. Serial No. 831,411.

*To all whom it may concern:*

Be it known that I, CARL T. FULLER, a citizen of the United States, residing at Nutley, county of Essex, State of New Jersey, have invented certain new and useful Improvements in the Treatment of Tungsten Filaments, of which the following is a specification.

My present invention relates to a method 10 of treating tungsten to increase its ductility and pliability and improve its capacity for retaining those properties after heating to the high temperatures of incandescence commonly employed in incandescent lamps and 15 similar devices.

It has been found that tungsten in the form of wire when prepared by the usual methods of manufacture heretofore employed, although ductile and pliable when 20 completed is so resilient that it is difficult to make it take a permanent set in a desired shape without heating and also that it loses some of its ductility after being maintained in the incandescent state for any consider- 25 able length of time.

I have discovered, however, that if tungsten wire is heated in the presence of an oxidizing agent under certain conditions it becomes so pliable as to readily take a per- 30 mament set without heating and that it retains its ductility for a longer period after heating to incandescence. The exact na- 35 ture of the action which takes place whereby the improved qualities of the wire are secured is not definitely known at the present time. It seems very likely however, that the oxygen acts to remove from the wire various impurities found therein in small amounts. These impurities may be present in the original metal and hence scattered throughout the entire mass or they may have been absorbed during the process of manu- 40 facture and confined to a thin surface layer of the wire.

In carrying my invention into effect if the wire is to be used for filaments, I may treat it after it has been mounted in the lamp by passing current through the lamp while it is connected to the evacuating pump and before the degree of vacuum at which the lamp is ordinarily sealed off has been reached. The small amount of oxygen present is sufficient to effect the desired improvement. Preferably, however, the completed wire is treated before it is mounted in the

lamps as more uniform results are obtained in this way. In this case the process may be made continuous by carrying the wire over two contacts in a partial vacuum or in an attenuated atmosphere of oxidizing gas and 60 passing current through it between the contacts to heat it to the desired temperature. It will also be understood that this latter method of treatment will be applicable 65 when the wire is to be used for other pur- poses than for filaments.

In the manufacture of filaments of ductile tungsten for incandescent lamps, difficulty has been experienced due to the tendency of 70 short sections of the filament to move lat- erally upon each other after prolonged heat- ing to incandescence and produce the condition known as "off-setting". Various meth- 75 ods of preparing tungsten have been de- vised, however, whereby this effect has been 80 avoided. For example, it has been found that if pure tungstic oxid is heated in a gas furnace in a covered Hessian or Battersea crucible it absorbs a small quantity of mat- ter consisting largely of alumina and silica 85 which probably is volatilized from the cruci- ble. The presence of from .8 to 1.5 of one per cent. of this additional matter intro- 90 duced at this stage of the refining of tung- 95 sten prevents offsetting of the completed 95 filament. It has also been found that the same result may be attained by adding to the tungsten small quantities of various refractory materials such as thorium oxid or thorium nitrate. My invention is especially 100 effective in connection with tungsten wire 105 which has been prepared by a process which results in non-offsetting filaments.

The most suitable temperature for pro- 105 ducing the desired results, the amount of the 95 oxidizing agent necessary and the length of time of heating the wire will vary. Gener- ally speaking it is believed that these factors depend upon the size of the wire and the 110 physical and chemical characteristics of the wire before treating and will have to be determined experimentally in each case. In order to enable one skilled in the art to practise my invention I will state however, that with a wire having a diameter of 1.2 105 mils which had been rendered non-offsetting by the addition of .75% of thorium oxid to the tungstic oxid from which it was pro- 110 duced I have obtained satisfactory results by passing the wire over two contacts spaced

one foot apart in a vacuum of 1-2 mm. of mercury at a rate of 10 feet per minute, and heating under these conditions to a temperature of approximately 1500 degrees C. Wire 5 thus treated, in addition to being less liable to be broken during the manufacture of the lamp, retains its ductility throughout a greater portion of the useful life of the lamp than wire which has not been subjected to 10 this process.

I have also obtained good results by first oxidizing the wire slightly, as for example by heating it to a dull red heat in the open air, and subsequently heating the oxidized 15 wire to a high temperature in a good vacuum, such as 1/10 mm. of mercury. The oxidized wire may be heated in an evacuated furnace or chamber, or it may be mounted to form the filament of an incandescent lamp 20 and then heated when the vacuum becomes sufficiently good during the exhaustion of the lamp. The temperature of the wire in the vacuum is increased gradually so that any tungsten oxid which is present will decompose without vaporizing or causing a 25 dark deposit on the lamp bulb.

I have also found that good results are obtained if tungsten wire suitably oxidized, as by heating in the open air, is subsequently 30 heated to the proper temperature in a suitable gas, such as nitrogen or forming gas, which is a mixture of nitrogen and hydrogen. If heated too hot while in the forming 35 gas the wire may become brittle. I have found that the oxidized wire can be heated

much higher with safety and that better results are obtained if the nitrogen or forming gas contains some air, or a large amount of water vapor, which may be introduced by bubbling the forming gas through water. 40

It will of course be understood that my invention is not limited to the treating of tungsten wire for use as filaments for incandescent lamps but that it will be of value in any case in which tungsten wire is to be 45 used for purposes where great strength, ductility and pliability are desirable and also where it is essential that these properties should be retained after prolonged heating to high temperatures. 50

What I claim as new and desire to secure by Letters Patent of the United States, is:—

1. The process of improving the mechanical properties of drawn tungsten wire which has been drawn by the usual methods of manufacture and which is later to be subjected to a temperature substantially higher than red heat, which consists in heating it to at least a red heat in an oxidizing atmosphere. 60

2. The process of treating drawn tungsten which consists in heating it to a high temperature in an attenuated atmosphere of an oxidizing agent.

In witness whereof I have hereunto set my 65 hand this 10th day of April, 1914.

CARL T. FULLER.

Witnesses:

S. N. WHITEHEAD,  
FRANK PARSONS.